

3,499,923

**POLYCHLOROALKYLPHOSPHONIC ACID SALTS**  
 Henryk A. Cyba, Evanston, Ill., assignor to Universal Oil  
 Products Company, Des Plaines, Ill., a corporation of  
 Delaware  
 No Drawing. Filed Sept. 7, 1965, Ser. No. 485,541  
 Int. Cl. C07c 69/40, 69/52, 69/60  
 U.S. Cl. 260—485

6 Claims

**ABSTRACT OF THE DISCLOSURE**

Polychloroalkylphosphonic acid salts of the condensation products of dialkanol amines and polycarboxylic acids or anhydrides, suitable for use as oxidation inhibitors.

This invention relates to a novel composition of matter and to the use thereof as an additive to organic substrates.

The novel composition of matter of the present invention is a trichloroalkylphosphonic acid salt of the condensation product of a dialkanol amine and a polycarboxylic acid or anhydride thereof.

The condensation product of dialkanol amine and dicarboxylic acid or anhydride is prepared in any suitable manner. Any suitable dialkanol amine is used as a reactant and will be selected with reference to the ultimate use of the salt. For example, when used, as an additive in lubricating oil or other organic substrates in which the additive is used in a concentration of greater than 1%, the dialkanol amine is an N-aliphatic dialkanol amine and preferably an N-alkyldialkanol amine in which the alkyl group contains at least 10 and preferably from about 10 to about 50 carbon atoms. However, when used as an additive in lower concentrations or for other uses, the alkyl group may contain a lesser number of carbon atoms. Illustrative N-alkyldiethanol amines include N-methyl - diethanolamine, N-ethyl - diethanolamine, N-propyl-diethanolamine, N-butyl-diethanolamine, N-amyl-diethanolamine, N-hexyl - diethanolamine, N - heptyl-diethanolamine, N - octyl - diethanolamine, N - nonyl-diethanolamine, N - decyl - diethanolamine, N - undecyl-diethanolamine, N-dodecyl - diethanolamine, N-tridecyl-diethanolamine, N-tetradecyl-diethanolamine, N-pentadecyl-diethanolamine, N-hexadecyl-diethanolamine, N-heptadecyl-diethanolamine, N-octadecyl-diethanolamine, N - nonadecyl - diethanolamine, N - eicosyl - diethanolamine, N - henei - cosyl - diethanolamine, N - docosyl-diethanolamine, N - tricosyl - diethanolamine, N - tetraicosyl - diethanolamine, N - pentacosyl - diethanolamine, N - hexacosyl - diethanolamine, N - heptacosyl - diethanolamine, N - octacosyl - diethanolamine, N - nonacosyl - diethanolamine, N - triacontyl - diethanolamine, etc.

It is understood that the N-aliphatic-diethanolamine may contain aliphatic substituents attached to one or both of the carbon atoms forming the ethanol group. These compounds may be illustrated by N-aliphatic-di-(1 - methyl - ethanolamine), N - aliphatic - di - (1-ethyl-ethanolamine), N-aliphatic - di - (1-propylethanolamine), N-aliphatic - di - (1-butylethanolamine), N-aliphatic-di-(1 - amylethanolamine, N - aliphatic - di - (1 - hexyl-ethanolamine), etc., N - aliphatic - di - (2 - methylethanolamine), N - aliphatic - di - (2 - ethylethanolamine), N - aliphatic - di - (2 - propylethanolamine), N - aliphatic - di - (2 - butylethanolamine), N - aliphatic - di - (2 - amylethanolamine), N - aliphatic - di - (2 - hexylethanolamine), etc. It is understood that these specific compounds are illustrative only and that other suitable compounds containing the diethanolamine configuration may be employed.

The specific compounds hereinbefore set forth are examples of N-aliphatic-diethanolamines. Other N-aliphatic-dialkanolamines include N - aliphatic - dipropanolamines and N-aliphatic-dibutanolamines, although N-aliphatic-dipentanolamines, N-aliphatic-dihexanolamines and higher dialkanolamines may be used in some cases. It is understood that these dialkanolamines may be substituted in a manner similar to that specifically described hereinbefore in connection with the discussion of the diethanolamines. Furthermore, it is understood that mixtures of N-aliphatic-dialkanolamines may be employed, preferably being selected from those hereinbefore set forth. Also, it is understood that the various dialkanolamines are not necessarily equivalent.

A number of N-alkyl-diethanolamines are available commercially and are advantageously used in preparing the condensation product. For example, N-tallow-diethanolamine is available under the trade name of "Ethomeen T/12." This material is a gel at room temperature, has an average molecular weight of 354 and a specific gravity at 25°/25° C. of 0.916. The alkyl substituents contain from about twelve to twenty carbon atoms per group and mostly sixteen to eighteen carbon atoms. Another mixed product is available commercially under the trade name of "Ethomeen S/12" and is N-soya-diethanolamine. It is a gel at room temperature, has an average molecular weight of 367 and a specific gravity at 25°/25° C. of 0.911. The alkyl substituents contain 16-18 carbon atoms per group. Still another commercial product is "Ethomeen C/12," which is N-coco-diethanolamine, and is a liquid at room temperature, and has an average molecular weight of 303 and a specific gravity at 25°/25° C. of 0.874. The alkyl groups contain mostly twelve carbon atoms per group, although it also contains groups having from eight to sixteen carbon atoms per group. Still another commercially available product is N-stearyl-diethanolamine, which is marketed under the trade name of "Ethomeen 18/12." This product is a solid at room temperature, has an average molecular weight of 372 and a specific gravity at 25°/25° C. of 0.959. It contains eighteen carbon atoms in the alkyl substituent.

Still another commercially available dialkanolamine is prepared by the oxyalkylation and more particularly by oxyethylation of beta-amines. The beta-amine is defined as an alkyl amine in which the nitrogen atom is attached to the second or beta carbon atom of the alkyl group. A commercially available diethanolamine in this embodiment is N - (1 - methyltetradecyl) - diethanolamine and is marketed under the trade name of "Ethomeen L-15/25." This diethanolamine has a melting point of about 50° F., a neutralization equivalent of 373 and a specific gravity at 25° C. of 0.897. It is understood that other dialkanolamines containing the beta configuration may be used. Illustrative examples include N - (1 - methyl - hexadecyl) - diethanolamine, N - (1 - methyl - heptadecyl) - diethanolamine, N-(1 - methyl - octadecyl) - diethanolamine, N - (1 - methyl - nonadecyl) - diethanolamine, etc., as well as corresponding dipropanolamines, dibutanolamines, etc. It is believed that these dialkanolamines may be of advantage in imparting to the final salt improved solubility in hydrocarbons and lower melting or softening points.

The N - aliphatic - dialkanolamine is reacted with a polycarboxylic acid. The polycarboxylic acid preferably comprises an aliphatic dicarboxylic acid. Illustrative dicarboxylic acids include oxalic, malonic, succinic, glutaric, adipic, pimelic, suberic, azelaic, sebacic, maleic, fumaric, itaconic, citraconic, mesaconic, etc. While the dicarboxylic acids are preferred, it is understood that polycarboxylic acids containing three, four, or more car-

boxylic acid groups may be employed. Furthermore, it is understood that a mixture of polycarboxylic acids and particularly of dicarboxylic acids may be used. A number of relatively inexpensive dicarboxylic acids comprising a mixture of these acids are marketed commercially under various trade names, including "VR-1 Acid," "Dimer Acid," "Empol 1022," etc., and these acids may be used in accordance with the present invention. For example, "VR-1 Acid" is a mixture of dicarboxylic acids and has an average molecular weight of about 700, is a liquid at 77° F., and has an acid number of about 150 and an iodine number of about 36. It contains thirty-six carbon atoms per molecule.

Another preferred polycarboxylic acid comprises a mixed acid being marketed commercially under the trade name of "Empol 1022." This dimer acid is a dilinoleic acid and is represented by the following general formula:



This acid is a viscous liquid, having an apparent molecular weight of approximately 600. It has an acid value of 180-192, an iodine value of 80-95, a saponification value of 185-195, a neutralization equivalent of 290-310, a refractive index at 25° C. of 1.4919, a specific gravity at 15.5°/15.5° C. of 0.95, a flash point of 530° F., a fire point of 600° F., and a viscosity at 100° C. of 100 centistokes. The above-mentioned "Dimer Acid" is substantially the same as "Empol 1022."

While the polycarboxylic acid may be employed, advantages appear to be obtained in some cases when using anhydrides thereof and particularly alkenyl-acid anhydrides. A preferred alkenyl-acid anhydride is dodecenylsuccinic anhydride. Other alkenyl-acid anhydrides include butenyl-succinic anhydride, pentenyl-succinic anhydride, hexenyl-succinic anhydride, heptenyl-succinic anhydride, octenyl-succinic anhydride, nonenyl-succinic anhydride, decenyl-succinic anhydride, undecenyl-succinic anhydride, tridecenyl-succinic anhydride, tetradecenyl-succinic anhydride, pentadecenyl-succinic anhydride, hexadecenyl-succinic anhydride, heptadecenyl-succinic anhydride, octadecenyl-succinic anhydride, nonadecenyl-succinic anhydride, eicosenyl-succinic anhydride, etc. While the alkenyl-succinic anhydrides are preferred, it is understood that the alkyl-succinic anhydrides may be employed, the alkyl groups preferably corresponding to the alkenyl groups hereinbefore specifically set forth. Similarly, while the aliphatic succinic anhydrides are preferred, it is understood that the anhydrides and particularly aliphatic-substituted anhydrides of other acids may be employed including, for example, adipic anhydride and particularly aliphatic adipic anhydrides, glutaric anhydride and particularly aliphatic glutaric anhydrides, etc.

It is understood that the aliphatic substituents attached to the N - aliphatic - dialkanolamine and/or the polycarboxylic acid or anhydride may be either of straight chain or branched chain configuration. Likewise, these aliphatic groups may be substituted by non-hydrocarbon groups including those containing nitrogen, oxygen, halogen and particularly chlorine and bromine, etc.

The condensation of N - aliphatic - dialkanolamine and polycarboxylic acid or anhydride is effected in any suitable manner but will comprise the inter-reaction with the liberation of water, and also may include the formation of a polymeric compound. The reaction generally is effected at a temperature above about 175° F. and preferably at a higher temperature, which usually will not exceed about 400° F., although higher or lower temperatures may be employed under certain conditions. The exact temperature will depend upon whether a solvent is used and, when employed, on the particular solvent. For example, with benzene as the solvent, the temperature will be of the order of 175° F., with toluene the temperature will be of the order of 250° F., and with xylene

the order of 300-320° F. Other preferred solvents include cumene, naphtha, Decalin, etc. Any suitable amount of the solvent may be employed but preferably should not comprise a large excess because this will tend to lower the reaction temperature and slow the reaction. Water formed during the reaction may be removed in any suitable manner including, for example, by operating under reduced pressure, by removing an azeotrope of water-solvent, by distilling the reaction product at an elevated temperature, etc. A higher temperature may be utilized in order to remove the water as it is being formed. The time of reaction is sufficient to effect the desired reaction and, in general, will range from about four to forty hours or more. Preferably one-half to two mole proportions of N - aliphatic - dialkanolamine are reacted with one mole proportion of acid.

The condensation product prepared in the above manner is reacted with a trichloroalkylphosphonic acid to form a salt. A preferred trichloroalkylphosphonic acid is trichloromethylphosphonic acid, which is available commercially, generally in the form of its monohydrate. The monohydrate may be used in forming the salt of the present invention. Other acids include trichloroethylphosphonic acid, trichloropropylphosphonic acid, trichlorobutylphosphonic acid, trichloropentylphosphonic acid, trichlorohexylphosphonic acid, as well as more highly chlorinated compounds as, for example, tetra, penta, hexa, or hepta chloroalkylphosphonic acids. Illustrative acids include pentachloroethylphosphonic acid, heptachloropropylphosphonic acid, etc. Here again it is understood that the hydrate of the acid may be used to prepare the salt of the present invention.

35 The salt is prepared in any suitable manner and generally by commingling the condensation product and acid, preferably with intimate stirring. Although the mixing may be effected at ambient temperature, generally it is preferred to heat the reaction mixture, usually at a temperature up to about 400° F. and preferably from about 175 to about 350° F. in order to facilitate formation of the salt. However, heating to an excessive temperature should be avoided in order to preclude chemical reaction between the acid and condensation product which would result in liberation of water, halogen or hydrogen halide.

In general the condensation product is used in a mole proportion of from 1 to 2 moles thereof per 1 mole of acid. However, it is understood that different proportions may be used which may range from 0.5 to 2 mole proportions of the condensation product per 1 mole proportion of acid. Stated another way, the condensation product is used in a proportion of from 0.5 to 2 basic equivalents per 1 acid equivalent of the trichloroalkylphosphonic acid.

55 Although applicant does not wish to be limited thereto, it is believed that the salt of the present invention will have the following configuration. The specific configurations set forth below describe the trichloromethylphosphonic acid salt of the condensation product of dodeceny succinic anhydride and Ethomeen T/12.



70 where  $n$  is an integer of from one to 100 and preferably from one to 10.

The above formula, when  $n$  is one, illustrates the condensation product of one hydroxyl of the diethanolamine with one anhydride oxygen. It is understood that the other hydroxyl groups of the diethanolamine can react with

another anhydride molecule and/or that the hydroxyl of the carboxyl groups may react with another diethanolamine molecule. This produces polyester type polymers which may be used in preparing the salts of the present invention.

A generic formula of the salt of the present invention may be represented by the following:



where R is an alkyl group of from 1 to 50 carbon atoms, R' is an alkylene group of from 2 to 8 carbon atoms, X is the residual fragment of the polycarboxylic acid, anhydride or further reaction product thereof, Y is hydrogen or COX, Z is the condensation product of the dialkanol amine and dicarboxylic acid or anhydride, n is an integer of from one to 100 and preferably from one to 10, and m is zero or one.

The salt may be recovered as a solid or viscous liquid but generally is in the form of a grease-like product. The salt may be utilized as such or dissolved in a suitable solvent and used in this manner. The solvent will be selected with reference to the use to be made of the salt. When the salt is to be used as an additive to hydrocarbon oil, a suitable solvent includes aromatic hydrocarbon and particularly benzene, toluene, ethylbenzene, cumene, or paraffin hydrocarbon including hexane, heptane, octane, nonane, etc., or mixtures containing one or both of these types of hydrocarbons such as naphtha, gasoline, kerosene, etc.

The salt of the present invention will have varied utility including use as an additive to organic substrates which undergo oxidative, thermal and/or other deterioration. Organic substrates include gasoline, naphtha, kerosene, jet fuel, lubricating oil, diesel fuel, fuel oil, residual oil, drying oil, grease, wax, resin, plastic, rubber, etc. In lubricating oil, the additive functions as a lubricity or extreme pressure agent. In addition, the additive serves as a flame-proofing agent, detergent-dispersant, peroxide decomposer, corrosion inhibitor, rust inhibitor, etc.

The salt of the present invention is advantageously used as an additive in lubricating oil. The lubricating oil may be of natural or synthetic origin. The mineral oils include those of petroleum origin and are referred to as motor lubricating oil, railroad type lubricating oil, marine oil, differential oil, diesel lubricating oil, gear oil, cylinder oil, specialty products oil, cutting oil, drawing oil, metal working lubricant, etc. Other oils include those of animal, marine or vegetable origin.

The lubricating oils generally have a viscosity within the range of from 10 SUS at 100° F. to 1000 SUS at 210° F. (SAE viscosity numbers include the range from SAE 10 to SAE 160). The petroleum oils are obtained from paraffinic, naphthenic, asphaltic or mixed base crudes. When highly paraffinic lubricating oils are used, a solubilizing agent also may be used if of advantage.

Synthetic lubricating oils are of varied types including aliphatic esters, polyalkylene oxides, silicones, esters of phosphoric and silicic acids, highly fluorine-substituted hydrocarbons, etc. Of the aliphatic esters di-(2-ethylhexyl) sebacate is being used on a comparatively large commercial scale. Other aliphatic esters include dialkyl azelates, dialkyl suberates, dialkyl pimelates, dialkyl adipates, dialkyl glutarates, etc. Specific examples of these esters include dihexyl azelate, di-(2-ethylhexyl) azelate, di-3,5,5-

trimethylhexyl glutarate, di-3,5,5-trimethylpentyl glutarate, di-(2-ethylhexyl) pimelate, di-(2-ethylhexyl) adipate, triamyl tricarboxylate, pentaerythritol tetracaproate, di-propylene glycol dipelargonate, 1,5-pentanediol-di-(2-ethylhexanone), etc. The polyalkylene oxides include polyisopropylene oxide, polyisopropylene oxide diether, polyisopropylene oxide diester, etc. The silicones include methyl silicone, methylphenyl silicone, etc., and the silicones include, for example, tetraisoctyl silicate, etc. The highly fluorinated hydrocarbons include fluorinated oil, perfluorohydrocarbons, etc.

Additional synthetic lubricating oils include (1) neopentyl glycol esters in which the ester group contains from three to twelve carbon atoms or more, and particularly neopentyl glycol propionates, neopentyl glycol butyrates, neopentyl glycol caproates, neopentyl glycol caprylates, neopentyl glycol pelargonates, etc., (2) trimethylol alkane esters such as the esters of trimethylol ethane, trimethylol propane, trimethylol butane, trimethylol pentane, trimethylol hexane, trimethylol heptane, trimethylol octane, trimethylol nonane, trimethylol decane, trimethylol undecane, trimethylol dodecane, etc., and particularly triesters in which the ester portions each contain from three to twelve carbon atoms and may be selected from those hereinbefore specifically set forth in connection with the discussion of the neopentyl glycol esters, (3) complex esters composed of dibasic acids and glycols, especially neopentyl, neohexyl, etc., glycols further reacted with monobasic acids or alcohols to give lubricants of viscosities at 210° F. of from four to twelve centistokes or higher, and (4) tricresylphosphate, trioctylphosphate, trinonylphosphate, tridecylphosphate, etc., as well as mixed aryl and alkyl phosphates.

The present invention also is used in the stabilization of greases made by compositing one or more thickening agents with an oil of natural or synthetic origin. Metal base synthetic greases are further classified as lithium grease, sodium grease, calcium grease, barium grease, strontium grease, aluminum grease, etc. These greases are solid or semi-solid gels and, in general, are prepared by the addition to the lubricating oil of hydrocarbon soluble metal soaps or salts of higher fatty acids as, for example, lithium stearate, calcium stearate, aluminum naphthenate, etc. The grease may contain one or more thickening agents such as silica, carbon black, talc, organic modified bentonite, etc., polyacrylates, amides, polyamides, aryl ureas, methyl N - n - octadecyl terephthalamate, etc. Another type of grease is prepared from oxidized petroleum wax, to which the saponifiable base is combined with the proper amount of the desired saponifying agent, and the resultant mixture is processed to a grease. Other types of greases in which the features of the present invention are usable include petroleum greases, whale grease, wool grease, etc., and those made from inedible fats, tallow, butcher's waste, etc.

etc. Oils of lubricating viscosity also are used as transmission fluids, hydraulic fluids, industrial fluids, etc., and the novel features of the present invention are used to further improve the properties of these oils. During such use the lubricity properties of the oil are important. Any suitable lubricating oil which is used for this purpose is improved by incorporating the additive of the present invention.

65 by incorporating the additive of the present invention. Oils of lubricating viscosity also are used as cutting oils, rolling oils, soluble oils, drawing compounds, etc. In this application, the oil is used as such or as an emulsion with water. Here again, it is desired that the oil serves to lubricate the metal parts of saws, knives, blades, rollers, etc., in addition to dissipating the heat created by the contact of the moving metal parts.

70 the contact of the moving metal parts.

Oils of lubricating viscosity also are used as slushing oils. The slushing oils are employed to protect finished or unfinished metal articles during storage or transportation from one area to another. The metal articles may be 75 of any shape or form including steel or other metal sheets,

plates, panels, coils, bars, etc., which may comprise machine parts, engines, drums, pistons rings, light arms, etc., as well as farm machinery, marine equipment, parts for military or other vehicles, household equipment, factory equipment, etc. A coating which may be visible to the eye, or not, as desired, covers the metal part and protects it from corrosion.

The salt of the present invention also is useful as an additive in fuel oil to prevent sediment formation. The fuel oil is marketed under various names including fuel oil, furnace oil, burner oil, range oil, diesel oil, etc. In such use the salt prevents sediment formation which may be due to oxidation, thermal reactions, etc., and also serves to disperse any sediment which is formed in the oil. The salt also serves as a rust or corrosion inhibitor, as well as retarding discoloration of the oil.

In another embodiment the salts of the present invention possess insecticidal properties with good inner-therapeutic action. They may be employed against many types of mites and insects such as, for example, Coraunius larvae, Cotoneaster aphid, apple aphid, black bean aphid, pea aphid, etc. The salt, preferably as a solution in a suitable solvent, may be used for the control of various larvae, mites, insects as flour beetle, Mexican bean beetle, black carpet beetle, milkweed bug, German cockroaches, southern army worms, mealy bug, sow bug, citrus red spider, greenhouse red spider, various mosquitoes, yellow fever mosquito, malarial mosquito, houseflies, etc.

As hereinbefore set forth, the salts of the present invention also possess flame-proofing or flame retardant properties and therefore, are useful in plastics, coatings, paints, drying oils, etc., as well as in fibrous materials. For example, in textiles, the salt imparts flame retardant as well as fungicidal properties to the fabric.

The concentration of the salt to be employed as an additive will depend upon the particular substrate in which it is to be used. In general, the additive is used in a concentration of from about 0.001% to about 25% by weight of the substrate and more specifically within the range of from 0.01% to about 5% by weight of the substrate. When used in conventional lubricating oil, the additive generally may be employed in a concentration of from about 0.01% to about 2% by weight of the oil. When used in lubricating oil for more severe operations, such as hypoid gear oil, the additive is used in a concentration of from about 1% to about 20% or more by weight of the oil. In general, substantially the same range of additive concentration is employed when the oil is used as transmission fluid, hydraulic fluid, industrial fluid, etc. When the oil is used in the formulation of a grease, the additive is used in a concentration of from about 0.5% to 5% by weight of the oil. When used in cutting oil, rolling oil, soluble oil, drawing compound, etc., the additive may be used in a concentration of from about 0.1% to about 10% by weight of the oil. When used in slushing oil, the additive may be used in a concentration of from about 0.1% to about 15% by weight or more of the oil.

It is understood that the additive of the present invention may be used along with other additives incorporated in the organic substrate. The other additives will depend upon the particular organic substrate. For example, in lubricating oil, the additional additives may comprise one or more of viscosity index improvers, pour point depressors, anti-foam additives, detergents, corrosion inhibitors, additional antioxidants, etc. Preferred additional antioxidants are of the phenolic type and include tertiary-butylcatechol, 2,6-ditertiarybutyl - 4 - methylphenol, 2,4-dimethyl-6-tertiarybutylphenol, etc., 2 - tertiarybutyl - 4-methoxyphenol, 2-tertiary-4-ethoxyphenol, 3,3',5,5'-tetra-tertiarybutyl-dihydroxydiphenylmethane, etc.

The salt of the present invention is an emulsifying agent and therefore will serve to emulsify water and oil of lubricating viscosity for use as lubricating oil, slushing oil, cutting oil, rolling oil, soluble oil, drawing com-

ound, etc. When desired, an additional emulsifying agent may be employed. Any suitable emulsifying agent can be used, including alkali metal sulfonates of petroleum sulfonic acids, mahogany sulfonates, naphthenic acids, fatty acids, etc., fatty alcohol sulfonates, pentaerythritol oleates, laurates, etc. The amount of water used in the emulsified oils will depend upon the particular use of the emulsion and may range from 0.25% to 50% or even up to 98% by weight of the composition.

The additive of the present invention is incorporated in the substrate in any suitable manner and preferably is suitably agitated with or otherwise mixed in the substrate in order to obtain intimate dispersion of the additive in the substrate. When the substrate comprises a mixture of two or more components, the additive of the present invention may be commingled with one of the components prior to mixing with the remaining component or components of the substrate.

The following examples are introduced to illustrate further the novelty and utility of the present invention but not with the intention of unduly limiting the same.

#### EXAMPLE I

The salt of this example is the trichloromethylphosphonic acid salt of the condensation product of dodecenyldsuccinic anhydride and Ethomeen T/12. As hereinbefore set forth, Ethomeen T/12 is N-tallow-diethanol amine in which the tallow group contains from 12 to 20 carbon atoms and mostly 16 to 18 carbon atoms per group.

The condensation product was prepared by refluxing 141 g. (0.5 mole) of dodecenyldsuccinic anhydride with 192 g. (0.5 mole) of Ethomeen T/12 in 100 g. of Decalin and 50 g. of xylene. The heating and refluxing were continued for a period of about 10 hours and a total of 10 cc. of water were collected. Following completion of the reaction, the reaction mixture was distilled under water pumped vacuum at about 380° F. to remove solvent. The condensation product was analyzed and found to have a basic nitrogen content of 1.60 meq./g. and a basic molecular equivalent weight of 625.

The salt was prepared by commingling 10.87 g. (0.1 equivalent or 0.05 mole) of trichloromethylphosphonic acid monohydrate with 62.5 g. (0.1 basic equivalent) of the condensation product of dodecenyldsuccinic anhydride and Ethomeen T/12 prepared as described above. The stirred mixture was heated to 195-212° F. and formed a homogeneous mixture. The mixture then was heated to about 265° F. to remove water which was present due to the use of the hydrate.

A 50% by weight solution of the salt in a commercial lubricating oil was prepared by adding 73 g. of a commercial lubricating oil to the salt prepared in the above manner and heating to about 250° F. with stirring. This resulted in a homogeneous solution, thereby demonstrating that the salt was soluble in the lubricating oil.

#### EXAMPLE II

The salt of the example is prepared by first forming the condensation product of maleic anhydride and Ethomeen T/12 and then reacting with trichloromethylphosphonic acid monohydrate.

The condensation product is prepared by refluxing 192 g. of Ethomeen T/12 (0.5 mole) and 49 g. (0.5 mole) of maleic anhydride in 200 g. of xylene. The heating and refluxing is continued for about 12 hours, during which time about 8.5 cc. of water is collected.

The salt is prepared by commingling, with stirring and heating, 110 g. (0.25 mole) of the condensation product prepared in the above manner and 78 g. (0.125 mole) of trichloromethylphosphonic acid monohydrate. The mixture is stirred and heated to a temperature of about 200° F. and then to a temperature of about 275° F. to remove water. The reaction mixture is allowed to cool to room temperature and the salt may be used as such but preferably is formed as a solution in a suitable solvent.

## EXAMPLE III

The salt of this example is prepared by first forming the condensation product of itaconic acid with Ethomeen C/12 and then reacting with trichloropropylphosphonic acid. The condensation product is prepared by heating and refluxing equal mole proportions of itaconic acid and Ethomeen C/12 in xylene solution. As hereinbefore set forth Ethomeen C/12 is N-coco-diethanol amine and is a liquid at room temperature, having an average molecular weight of 303 and containing an average of 12 carbon atoms per alkyl group. The heating and refluxing is continued until the theoretical amount of water is recovered. After cooling to room temperature, an equal mole proportion of trichloropropylphosphonic acid is added to the condensation product and the mixture is mixed and heated to 180° F. to insure complete forma-

5

10

15

In another series of tests the machine was operated for five minutes at each load from 250 pounds to seizure at 250 pound increments. The maximum load and the time in minutes at this load to seizure are reported, as well as the temperature of the oil. In this case the higher temperature is preferred because it means that the oil is operating satisfactorily at a high temperature.

The lubricating oil used in this example is dioctyl sebacate synthetic lubricating oil marketed under the trade name of "Plexol 201."

Run No. 1 in the following table is a run made using the "Plexol" not containing an additive and thus is the blank or control run.

Run No. 2 is a run made using another sample of the "Plexol" to which has been added 4% by weight of the solution prepared as described in Example I (2% by weight of active ingredient).

TABLE I

| Run No. | Temperature, ° F. |     |       | Torque, lbs. |       |       | Wear, teeth |     |     | Seizure conditions |      |            |
|---------|-------------------|-----|-------|--------------|-------|-------|-------------|-----|-----|--------------------|------|------------|
|         | 250               | 500 | 750   | 250          | 500   | 750   | 250         | 500 | 750 | Load               | Time | Temp. ° F. |
| 1-----  | 150               | 231 | 490-S | 3-4          | 9-10  | 18-S  | 0           | 0   | S   | 750                | 2    | 490        |
| 2-----  | 151               | 257 | 363   | 4-5          | 13-14 | 16-24 | 0           | 0   | 12  | 2,000              | 2    | 600        |

S—Seizure.

tion of the salt. The salt is recovered in solution in the xylene solvent and the solution is used as an additive to organic substrates.

## EXAMPLE IV

The salt of this example is prepared in substantially the same manner as described in the previous preparations by first forming the condensation product of N-decyl-dipropanol amine and dilinoleic acid and then reacted with trichloroethylphosphonic acid. For economical reasons, the acid used in Empol 1022 which is available commercially. The properties of this acid have been set forth hereinbefore. The N-decyl-dipropanol amine and dilinoleic acid are heated and refluxed in the presence of toluene solvent until the theoretical amount of water is liberated. The condensation product is then reacted with trichloroethylphosphonic acid, with stirring and heating, to form the salt.

## EXAMPLE V

As hereinbefore set forth the salt of the present invention is of special utility in lubricating oil. One method of evaluating lubricating oils is by the Falex machine. This procedure is described in detail in a book entitled "Lubricant Testing" authored by E. G. Ellis and published by Scientific Publications (Great Britain) Limited, 1953, pages 150-154. Briefly, the Falex machine consists of a rotating pin which runs between two "V" shape bearings which are spring loaded against the pin and provided with means for varying the load. The oil to be tested is poured into a metal trough in which the pin and bearings are partly submerged. The machine was operated for five

30

35

40

45

50

55

From the data in the above table it will be seen that the dioctyl sebacate without additive (Run No. 1) underwent seizure at a load of 750 pounds. In contrast, seizure conditions for the example of the dioctyl sebacate containing the additive of the present invention was 2000 pounds. As another advantage to the additive of the present invention, the oil did not undergo darkening during Run No. 2.

## EXAMPLE VI

Another series of evaluations was made in the same manner as described in Example V, except that the lubricating oil was a mineral oil marketed commercially as "Carnes 340 White Oil." Typical specifications of this oil include the following:

|                            |      |         |
|----------------------------|------|---------|
| Distillation range         | ° F. | 740-975 |
| Specific gravity at 60° F. |      | 0.8836  |
| Viscosity:                 |      |         |
| At 100° F.                 |      | 360     |
| At 210° F.                 |      | 52.2    |
| Flash point, COC           | ° F. | 440     |
| Pour point                 | ° F. | -20     |
| Refractive index at 68° F. |      | 1.4805  |
| Saybolt color              |      | +30     |

Run No. 3 in the following table is a run using the white oil not containing an additive and thus is the blank or control run.

Run No. 4 is a run using another sample of the white oil to which has been added 4% by weight of the salt solution prepared as described in Example I (2% by weight of active ingredient).

TABLE II

| Run No. | Temperature, ° F. |       |       | Torque, lbs. |       |       | Wear, teeth |     |       | Seizure conditions |      |            |
|---------|-------------------|-------|-------|--------------|-------|-------|-------------|-----|-------|--------------------|------|------------|
|         | 250               | 500   | 750   | 250          | 500   | 750   | 250         | 500 | 750   | Load               | Time | Temp. ° F. |
| 3-----  | 172               | 350-S | ----- | 5-6          | 30-S  | ----- | 0           | S   | ----- | 425                | 0.1  | 275        |
| 4-----  | 164               | 277   | 413   | 4-5          | 13-15 | 19-22 | 0           | 0   | 24    | 2,000              | 2    | 650        |

S—Seizure.

minutes each at 250 and 500 pound loads and then for forty-five minutes at 750 pound load. The data collected includes the temperature of the oil and the torque at each of the loads, as well as the wear which is determined by a ratchet wheel arrangement in which the teeth are advanced in order to maintain the desired load. Each tooth is equivalent to approximately 0.000022 inch. Preferred additives are those which impart low temperature, low torque and low wear to the oil.

70

75

Here again it will be seen that the oil without additive (Run No. 3) underwent seizure at a small load, in this case of 425 pounds. In contrast, the oil containing the additive of the present invention did not undergo seizure until a load of 2000 pounds.

## EXAMPLE VII

The salt solution prepared as described in Example I also was evaluated as a sediment inhibitor in fuel oil.

This evaluation was made according to the "Erdco" test in which heated oil is passed through a filter and the time required to develop a differential pressure across the filter of 25 in. Hg is determined. It is apparent that the longer the time, the more effective is the additive. However, with a very effective additive, the time to reach a differential pressure across the filter of 25 in. Hg is lengthened beyond reasonable limits that the test is stopped after about 300 minutes and the differential pressure at that time is reported.

In this evaluation, 0.001% by weight of the solution prepared as described in Example I was incorporated in a commercial range oil and evaluated in the Erdco test. A differential pressure of only 0.4 in. Hg after 300 minutes was developed, in contrast to a differential pressure of 25 in. Hg in less than 100 minutes for a sample of the oil not containing the additive.

#### EXAMPLE VIII

The salt prepared as described in Example III is used in a concentration of 1% by weight as an additive in grease. The additive is incorporated in a commercial Mid-Continent lubricating oil having an S.A.E. viscosity of 20. Approximately 92% of the lubricating oil then is mixed with approximately 8% by weight of lithium stearate. The mixture is heated to about 450° F., with constant agitation. Subsequently, the grease is cooled, while agitating, to approximately 248° F., and then the grease is further cooled slowly to room temperature.

The stability of the grease is tested in accordance with ASTM D-942 method, in which method a sample of the grease is placed in a bomb and maintained at a temperature of 212° F. Oxygen is charged to the bomb, and the time required for a drop of five pounds pressure is taken as the Induction Period. A sample of the grease without additive will reach the Induction Period in about eight hours. On the other hand, a sample of the grease containing 1% by weight of the additive of the present invention will be of substantially higher stability.

I claim as my invention:

1. Polychloroalkylphosphonic acid salt of the condensation product of dialkanol amine and polycarboxylic acid or anhydride thereof, said dialkanol amine having

from 2 to about 6 carbon atoms in each of the alkanol groups and said acid being selected from the group consisting of oxalic, malonic, succinic, glutaric, adipic, pimelic, suberic, azelaic, sebacic, maleic, fumaric, itaconic, citraconic and mesaconic acids, said salt containing from 5 3 to 7 chlorine atoms and the alkyl group thereof containing from 1 to 6 carbon atoms.

2. The acid salt of claim 1 further characterized in that said dialkanol amine is an N-alkyl dialkanol amine 10 having from 1 to 50 carbon atoms in the alkyl group.

3. Trichloromethylphosphonic acid salt of the condensation product of from 1 to 2 mole proportions of an N-alkyl diethanol amine in which said alkyl group contains from 1 to 50 carbon atoms with a dicarboxylic acid or anhydride thereof, said acid being selected from the group consisting of oxalic, malonic, succinic, glutaric, adipic, pimelic, suberic, azelaic, sebacic, maleic, fumaric, itaconic, citraconic and mesaconic acids.

4. Trichloromethylphosphonic acid salt of the condensation product of from 1 to 2 mole proportions of N-tallow diethanol amine with 1 mole proportion of polycarboxylic acid or anhydride thereof, said acid being selected from the group consisting of oxalic, malonic, succinic, glutaric, adipic, pimelic, suberic, azelaic, sebacic, maleic, fumaric, itaconic, citraconic and mesaconic acids.

5. Trichloromethylphosphonic acid salt of the condensation product of from 1 to 2 mole proportions of N-tallow diethanol amine with dodecetyl-succinic anhydride.

6. Trichloromethylphosphonic acid salt of the condensation product of from 1 to 2 mole proportions of N-tallow diethanol amine with maleic anhydride.

#### References Cited

##### UNITED STATES PATENTS

2,882,228 4/1959 Watson et al. ----- 250—56

LORRAINE A. WEINBERGER, Primary Examiner

E. J. SKELLY, Assistant Examiner

U.S. CL. X.R.

44—71; 252—32.5, 356, 8.1, 389; 260—999, 45.85